# EUROPEAN PATENT SPECIFICATION

(11) **EP 2 977 487 B1**
(45) Date of publication and mention of the grant of the patent: **05.09.2018**
(21) Application number: 14178573.3
(22) Date of filing: 25.07.2014
(51) Int. Cl.: C23C 24/08, C23C 28/04, C04B 41/00, F01D 5/28

(54) **Method for smoothing the surface of a coating**
Verfahren zur Glättung der Oberfläche einer Beschichtung
Procédé pour lisser la surface d'un revêtement

(43) Date of publication of application: 27.01.2016
(73) Proprietor: Ansaldo Energia IP UK Limited, London W1G 9DQ (GB)
(72) Inventor: Renusch, Daniel, 5400 Baden (CH); Witz, Gregoire Etienne, 5413 Birmenstorf (CH); Bossmann, Hans-Peter, 79787 Lauchringen (DE)
(74) Representative: Bernotti, Andrea

(56) References cited:
- EP-A1- 2 236 650
- EP-A2- 1 088 908
- EP-A2- 2 287 129
- WO-A1-2009/030049

## Description

### BACKGROUND OF THE INVENTION

The present invention relates to a method for smoothing the rough surface of thermal barrier coatings (TBC's) which are used for protection of thermal high loaded components, such as gas turbine blades, vanes or combustor parts.

### PRIOR ART

Above mentioned surfaces of coatings exhibit a certain roughness. Within the meaning of the present application, smoothing the surface of the coating means that the roughness of said surface is reduced.

It is known state of the art to use TBC's for improvement of the performance of metallic components which are exposed to high temperatures.

Although gas turbine components are made of alloys, for example Ni-, Co- or Fe-based superalloys, which can resist high temperatures of more than 1000 °C there is a need for further increasing the operating temperature of the turbines to improve the efficiency of the gas turbines. This can be achieved among others for example by applying a thermal barrier coating onto the surface of the superalloy component. Most of the applied TBC's are ceramic-based coatings, preferably yttria-stabilized zirconia (YSZ). Such a material has a much higher temperature resistance than the above mentioned superalloys.

The TBC's are usually applied by thermal spray techniques, such as plasma spray processes like APS (Air/Atmospheric Plasma Spraying), VPS (Vacuum Plasma Spraying) or the very expensive EB-PVD (Electron Beam Physical Vapor Deposition).

APS technique is cheaper with respect to EB-PVD, but it has the disadvantage of a relative rough surface which can cause problems with respect to aerodynamic drag losses of appropriate coated gas turbine components. During operation of a gas turbine surface roughness increases turbulent heat transfer from the hot combustion gases to the component and thus reduces aerodynamic performance.

Therefore, several methods are used for smoothing the surface of the coatings, for example mechanical methods like grinding, polishing or sandblasting. Those methods can have the disadvantage of damaging the surface.

Additionally, the efficacy of the TBC is improved by introducing porosity in to the coating. However, when polishing the TBC, this inherent porosity will place a limit on the smoothness. The polishing process can open the closed pores.

Another method is described in document US 7368164 B2. A component used in a high-temperature environment, such as the combustor section of a gas turbine, is coated with a TBC made of yttria-stabilized zirconia, which provides the thermal protection for the substrate of the component. A bond coat, for example made of MCrAlY, is applied between the substrate and the TBC to promote adhesion of the TBC. The TBC is sprayed onto the bond coat by APS which results in a certain degree of inhomogeneity and porosity and in a rough surface of about 5-13 µm Ra. This leads to problems with respect to erosion resistance, transmissivity to infrared radiation and aerodynamic performance. To overcome these drawbacks the TBC is over-coated by a multilayer outer coating which is formed of two layers having different compositions. An inner layer of the coating contains alumina in a first silica-containing matrix material that is free of zinc titanate. An outer layer of the coating contains alumina, a glass material and zinc titanate in a second silica-containing matrix material. The thickness, structure and properties of the outer coating can be tailored by the firing temperature and durations used for each inner and outer layer. The outer layer of the coating has a low surface roughness Ra< 3 µm and forms the outermost surface of the component. As a result the new coating reduces the component temperature by reducing the convective and radiant heat transfer thereto. But the deposition of two different layers to the underlying TBC is expensive.

US 2007/0099013 A1 discloses also a method for manufacturing a TBC coated machine component, wherein a "smooth coat" ceramic layer is applied onto the component subsequent to the TBC. Because some of these smooth coat materials do not have a good adherence to the underlying TBC the smooth coat layer may spall during curing. To overcome the chipping of the smooth layer it is proposed in this document to deposit two TBC's, the outer thermal barrier coating having a higher porosity than the inner one, such to reduce the risk of delamination of the smooth coating layer. Such a solution is also cost intensive due to the necessity to deposit two different layers of TBC that means an additional layer of TBC is required.

Documents US 6294261 B1, EP 1088908 A2, EP 2236650 A1 describe further methods respective smooth slurry/gel layers or multilayer coatings to be deposited on a TBC. US 6294261 B1 and. EP 1088908 A2 disclose for example a slurry/gel composition which is based on yttria-stabilized zirconia as refractory filler and precursors of an oxide matrix, for example an alumina or an aluminosilicate matrix. The method for smoothing the surface of the protective coating (YSZ TBC) includes the steps of applying the slurry/gel to the TBC surface, heating the slurry/gel coating to remove volatile material and then further heating to cure the coating and bond it to the underlying protective coating. Using a slurry comprising zirconia means a good match of the thermal expansion coefficient of the TBC and the smooth layer. Matching the composition is a good way to reduce the thermo-mechanical stresses, but if the coating is too thick it will not prevent the formation of vertical cracks in the smooth layer. Unfortunately, such cracks reduce the aerodynamic efficiency of the smooth coating reducing the benefit of the coating.

The challenge according to those documents is to provide a smooth layer that has a low roughness (Ra< 6 µm, preferentially <3 µm) without reducing the lifetime of the underlying thermal barrier coating. The roughness that can be achieved with the smooth layer is strongly affected by the layer porosity. Therefore a low porosity in the coating prior to polishing (< 1 %) is necessary. At low coating porosity the coating is stiff with a high Young's modulus. Due to this high modulus, thermo-mechanical stresses linked to the difference in the coefficient of thermal expansion between the smooth layer and the underlying TBC can be sufficient to induce cracking in one or both coatings. Depending on the coating architecture this can lead either to early TBC spallation or to smooth layer chipping and reduction of the aerodynamic performance.

### SUMMARY OF THE INVENTION

It is an object of the present invention to provide an effective and cost-efficient method for smoothing the surface of a coating that means reducing the roughness Ra of a ceramic TBC which is applied to a high thermally loaded gas turbine component made of a superalloy.

It is another object of the disclosure to disclose an appropriate smooth coating system itself, comprising a TBC which is used for protection of gas turbine components and which improves the aerodynamic behavior and therefore increases the turbine efficiency and which is able to minimize the thermo-mechanical stresses.

These and other objects are obtained by a method according to claim 1. The disclosed method for reducing the roughness of a first coating with a defined coating composition and a thermal expansion coefficient, said coating covering the surface of a component to be thermally high loaded, comprises that
- in a first step the roughness of said coating is measured and
- in a following step a second slurry coating is prepared for applying onto the surface of the first coating, whereby the coating composition of the second coating is tailored to have a similar thermal expansion coefficient like the first coating. The method is characterized in
- calculating a minimum number of coating spray passes necessary to provide the second slurry coating with a thickness that is at least two times the surface roughness of the first coating;
- applying the slurry coating with said calculated number of passes onto the surface of the first coating;
- fully curing, but only partially sintering the slurry coating at a temperature in the range of 300 to 800 °C and
- polishing the second coating to reduce the thickness such that finally the second coating does cover the first coating only locally.

The last mentioned step is done by polishing the slurry down to the point where the "peaks" in the underlying TBC roughness are at the surface (visibly), and only the "valleys" in the TBC roughness remain filled with slurry coating.

With such a technical solution a dense, thin coating for a smooth layer can be provided to minimize the thermo-mechanical stresses using a cost effective manufacturing process. Minimizing the smooth layer thickness and polishing it such that the smooth layer (= second coating) does not cover 100 % of the first coating surface after smoothening it, leaving some areas where the first coating is appearing.

To achieve such a low smooth layer thickness without requiring a long time and cost consuming polishing process, the coating has to be manufactured such that it is dense, fully cured but only partially sintered to avoid too much recrystallization of the filler material. In this state the slurry coating can be described as a "machinable ceramic".

According to an embodiment of the invention the curing resp. partially sintering of the slurry coating is done at a temperature in the range of 500 to 800 °C. The slurry coating is a zirconia based slurry coating with a small amount of alumina silicate or zirconium silicate. The zirconia can be un-stabilized or preferably stabilized, more preferably stabilized with Y₂O₃, CaO, MgO or any combinations thereof. The slurry coating binder is a silicate solution, phosphate solution or silicon emulsion. The first coating is a ceramic thermal barrier coating (TBC), preferably made of chemically stabilized zirconia. By using those materials it is realized that the thermal expansion coefficients of both coatings are close to each other.

The described method is for coating systems where the first coating is applied by atmospheric plasma spraying and has therefore a relative high roughness and high porosity, which can cause the above described disadvantages, for example reduction of aerodynamic performance.

The disclosed coating system for surface protection of a thermally high loaded component which is produced with a method according to claims 1 is characterized in that the coating system consists of a first underlying coating and a second slurry coating overlaying the first coating, wherein both coatings (1, 2) have a chemical composition with a similar thermal expansion coefficient, and wherein the second coating is very dense with a porosity < 1%, fully cured, but only partly sintered and wherein the second coating does only cover locally the first coating, so that said coating system finally comprises a reduced roughness with respect to the roughness of the originally applied first coating. The coating system for surface protection of a thermally loaded component has a second coating which is only completely sintered as a result of the first firing in the engine. The disclosed coating system is applied onto the surface of a gas turbine component made of a Ni-, Co-, Fe-based superalloy or combinations thereof, wherein the first coating is a ceramic thermal barrier coating, preferably made of chemically stabilized zirconia and the second coating is made by applying of a zirconia based slurry.

### BRIEF DESCRIPTION OF THE DRAWINGS

The present invention is now to be explained more closely by means of different embodiments and with reference to the attached drawings.
- Fig. 1: shows a typical cross section of a TBC as first coating and a very thin smooth layer (second coating) according to an embodiment of the present invention;
- Fig. 2: shows schematically the results after different steps (2a-2c) of the disclosed method;
- Fig. 3: shows the surface of a coating in service in form of a photo, when the coating is too thick (prior art) and
- Fig. 4: shows the surface of a coating in form of a photo, where the coating was manufactured according to the present invention.

### DETAILED DESCRIPTION OF DIFFERENT EMBODIMENTS OF THE INVENTION

The present invention is related to a method for smoothing the rough surface of thermal barrier coatings (TBC's) which are used for protection of thermal high loaded components, such as gas turbine blades, vanes or combustor parts.

TBC's especially applied by atmospheric plasma spraying methods onto the surface of above mentioned components have a relative high roughness. For improving the aerodynamic behavior which allows increasing the turbine efficiency it is necessary to provide a smooth surface layer by an efficient method which is cheaper and faster with respect to the known methods in the prior art. Additionally, to improve perform in-service the smooth surface layer needs to be thinner.

The present application discloses a method for reducing the roughness Ra of a first coating 1 with a defined coating composition and a thermal expansion coefficient, said coating 1 covering the surface of a component 3 to be thermally high loaded, the method comprises that in a first step the roughness of said coating 1 is measured and in a following step a second slurry coating 2 is prepared for applying onto the surface of the first coating 1, whereby the coating composition of the second coating 2 is tailored to have a similar thermal expansion coefficient like the first coating 1. The method is characterized in
- calculating a minimum number of coating spray passes N necessary to provide the second slurry coating 2 with a thickness T that is at least two times of the roughness of the first coating 1,
- applying the slurry coating 2 with said calculated number of spray passes N onto the surface of the first coating 1;
- fully curing, but only partially sintering the slurry coating 2 at a temperature in the range of 300 to 800 °C and
- polishing the second coating 2 to a reduced thickness T' such that finally the second coating 2 does cover the first coating 1 only locally (i.e. The "valleys" in the underlying TBC roughness are filled with dense slurry.).

With such a technical solution a dense coating 2 for a smooth layer can be provided to minimize the thermo-mechanical stresses using a cost effective manufacturing process. Minimizing the smooth layer thickness T and polishing it to a reduced thickness T' such that the smooth layer (= second coating 2) does not cover 100 % of the first coating's 1 surface after smoothening it, leaving some areas where the first coating 1 is appearing.

To achieve such a low smooth layer thickness without requiring a long time and cost consuming polishing process, the coating has to be manufactured such that it is dense, fully cured, but only partially sintered to avoid too much recrystallization of the filler material.

According to an embodiment of the invention the curing resp. partially sintering of the slurry coating is done at a temperature in the range of 500-800 °C.

Fig. 1 shows a photo of the microstructure (cross section) of a typical TBC 1 with a smooth layer 2 on the top according to one embodiment of the invention, where the desired reduction in surface roughness is achieved. The smooth layer 2 is very thin to the extent that the slurry fills the "valleys" in the underlying TBC roughness.

The "peaks" in the underlying TBC roughness are not covered by the slurry coating. The slurry is in the "valleys" of the underlying TBC roughness. The "peaks" in the underlying TBC roughness are not covered by the slurry coating.

The embodiment in Fig. 1 is a component produced with the method according to the present disclosure. The component is made of Hastelloy X base material. It has an APS MCrAlY bond coat. The TBC (first coating 1) is APS 7 wt% yttria-stabilized zirconia. The slurry coating (second coating 2) is un-stabilized zirconia with the addition of a small amount of alumina silicate. The slurry coating binder was a water based silicon emulsion. The average initial TBC roughness Ra was 17.2µm. The average initial TBC thickness was 941µm, measured non-destructively with eddy-current equipment. The slurry coating was applied with a commercial paint sprayer. The number of spray passes N was 6. The eddy-current thickness measurements of the as sprayed slurry plus the TBC had an average value of 982 µm, thus the average slurry coting 2 thickness T was 41µm. The slurry was cured at 700°C for 5h. After curing the slurry coating 2 was polished with a fine grit wet silicon-carbide paper. After polishing the finial average roughness Ra' was found to be 2.8 µm. The non-destructive eddy-current thickness measurements of the as smooth layer plus the TBC had an average value of 945 µm. From the cross section photos the deepest slurry filed "valley" depth was 21µm.

The partially sintered slurry coating 2 is inherently softer than the TBC coating 1. During the beginning of polishing of the softer slurry coating, the abrasion rate is relatively high. As the slurry coating becomes thinner and the tops of the harder TBC "peaks" in the roughness are reached the polishing abrasion rates slows and even stops. Thus leaving only the TBC "valleys" in the roughness are filled with the slurry coating. The zirconia based slurry coating has a small amount of alumina silicate or zirconium silicate. The zirconia can be unstabilized or stabilized with Y₂O₃, CaO, MgO or any combinations thereof. The slurry coating binder is a silicate solution, phosphate solution or silicon emulsion. The first coating is a ceramic thermal barrier coating (TBC), preferably made of chemically stabilized zirconia. By using those materials it is realized that the thermal expansion coefficients of both coatings are close to each other.

The described method is effective for coating systems where the first coating is applied by atmospheric plasma spraying and has therefore a relative high roughness, which can cause the above described disadvantages, for example reduction of aerodynamic performance.

The disclosed coating system or surface protection of a thermally high loaded component which is produced with a method according to claims 1 is characterized in that the coating system consists of a first underlying coating and a second slurry coating overlaying the first coating, wherein both coatings 1, 2 have a chemical composition with a similar thermal expansion coefficient, and wherein the second coating is very dense with a porosity < 1%, fully cured, but only partly sintered and wherein the second coating does only cover locally the first coating, so that said coating system finally comprises a reduced roughness with respect to the roughness of the originally applied first coating. The coating system for surface protection of a thermally loaded component has a second coating which is only completely sintered as a result of the first firing in the engine. The disclosed coating system is applied onto the surface of a gas turbine component made of a Ni-, Co-, Fe-based superalloy or combinations thereof, wherein the first coating is a ceramic thermal barrier coating, preferably made of chemically stabilized zirconia and the second coating is made by applying of a zirconia based slurry.

Fig. 2 shows schematically the results after different steps of the disclosed method.

Fig. 2a shows the first coating 1 prior to the applying of the second coating - the high roughness Ra is clearly to be seen, it is about 8-18 µm.

Fig. 2b shows the system with the first coating 1 and the applied second coating 2. The roughness of the first coating Ra is the same like in Fig. 2a, but the overlying coating 2 may provide a smooth surface however it is too thick (with an average thickness T≥2xRa) and may crack during serves.

Fig. 2c shows the result after the last step of the described method according to claim 1. The coating system comprises the first coating 1 with the second coat 2 and a reduced roughness Ra' (which is about 1-6 µm) with respect to the originally applied coating 1. The reduced thickness T' of the second coating 2 is T'≈ Ra, such that finally the second coating 2 does cover the first coating 1 only locally.

According to an embodiment of the invention, the number of spray passes N, the thicknesses T, T' and roughness Ra, Ra' are coupled, by approximately N ≥ T/R (with R= deposition rate for one spray pass N), T ≥ 2xRa, after smoothing T' ≈ Ra, which may require optimizing for special composition and coating equipment.

Fig. 3 shows in a photo the surface of a coating in service, when the smooth surface coating is too thick (prior art). A lot of undesired cracks can be recognized.

In contrast to Fig. 3 Fig. 4 shows in a photo the surface of a coating system manufactured according to the present invention. The dark spots are the TBC appearing at the surface after the polishing step. Microcracks / cracks can't be recognized. The dark spots are the "peaks" in the underlying TBC roughness appearing at the surface.

The durability of the coating is ensured, providing improved aerodynamic performance over a long period of operation. There is also no thermal barrier coating lifetime reduction due to the smoothened surface.

### List of reference numerals

- 1: first coating, preferably TBC
- 2: second coating, slurry coating
- 3: thermally loaded component, for example gas turbine blade
- 4: coating system
- Ra: roughness of the surface (of the first coating 1)
- Ra': reduced final roughness of the surface
- T: thickness of pos. 2
- T': reduced thickness of pos. 2
- N: number of coating spray passes for pos. 2
- R: deposition rate for one spray pass

## Claims

1. Method for reducing the roughness (Ra) of a ceramic thermal barrier coating (1) with a defined coating composition and thermal expansion coefficient, said ceramic thermal barrier coating (1) covering the surface of a Ni-, Co-, Fe-based superalloy component (3) of a gas turbine to be thermally high loaded, wherein:
- in a first step the ceramic thermal barrier coating (1) is applied onto the surface of a component (3) by atmospheric plasma spraying and the roughness (Ra) of said ceramic thermal barrier coating (1) is measured and
- in a following step a zirconia based slurry coating (2) with alumina silicate or zirconium silicate additives and a slurry coating binder being a silicate solution, phosphate solution or silicon emulsion is prepared for applying onto the surface of the ceramic thermal barrier coating (1), the coating composition of the zirconia based slurry coating (2) being tailored to have a similar thermal expansion coefficient like the ceramic thermal barrier coating (1);
- calculating a minimum number of coating spray passes (N) necessary to provide the zirconia based slurry coating (2) with a thickness (T) that is at least two times of the roughness (Ra) of the ceramic thermal barrier coating (1),
- applying the zirconia based slurry coating (2) with said calculated number of spray passes (N) onto the surface of the ceramic thermal barrier coating (1);
- fully curing, but only partially sintering the zirconia based slurry coating (2) at a temperature in the range of 300 to 800°C;
- polishing the zirconia based slurry coating (2);
- completely sintering the zirconia based coating (2) only after the first exposition to thermal loaded operation of the component (3);
the polishing step is performed until the peaks of the roughness (Ra) are reached so the thickness (T) of the zirconia based slurry coating (2) becomes a reduced thickness (T') substantially equal to the roughness (Ra) of the ceramic thermal barrier coating (1) such that finally the zirconia based slurry coating (2) does cover the ceramic thermal barrier coating (1) only locally at the valleys of the roughness (Ra).

2. Method according to claim 1, **characterized in** curing resp. partially sintering the slurry coating (2) at a temperature in the range of 500 to 800 °C.

3. Method according to claim 1, **characterized in that** the zirconia is stabilized with Y₂O₃, CaO, MgO or any combinations thereof.

4. Method according to claim 1, **characterized in that** the ceramic thermal barrier coating (1) is made of chemically stabilized zirconia.

## Patentansprüche

1. Verfahren zum Verringern der Rauheit (Ra) einer keramischen Wärmesperrbeschichtung (1) mit einer definierten Beschichtungszusammensetzung und einem definierten Wärmeausdehnungskoeffizienten, wobei die keramische Wärmesperrbeschichtung (1) die Oberfläche einer Ni-, Co- und Fe-basierten Superlegierungskomponente (3) einer Gasturbine, die stark wärmebelastet werden soll, abdeckt, wobei
- in einem ersten Schritt die keramische Wärmesperrbeschichtung (1) durch atmosphärisches Plasmaspritzen auf die Oberfläche einer Komponente (3) aufgebracht wird und die Rauheit (RA) der keramischen Wärmesperrbeschichtung (1) gemessen wird und
- in einem folgenden Schritt eine zirkonoxidbasierte Aufschlämmungsbeschichtung (2) mit Aluminiumoxidsilikat- oder Zirkoniumsilikat-Zusatzstoffen und einem Aufschlämmungsbeschichtungsbindemittel, das eine Silikatlösung, eine Phosphatlösung oder eine Siliziumemulsion ist, zum Aufbringen auf die Oberfläche der keramischen Wärmesperrbeschichtung (1) angefertigt wird, wobei die Beschichtungszusammensetzung der zirkonoxidbasierten Aufschlämmungsbeschichtung (2) zugeschnitten ist, einen ähnlichen Wärmeausdehnungskoeffizienten wie die keramische Wärmesperrbeschichtung (1) zu besitzen;
- Berechnen einer Mindestzahl von Beschichtungsspritzdurchgängen (N), die erforderlich ist, um die zirkonoxidbasierte Aufschlämmungsbeschichtung (2) mit einer Dicke (T), die mindestens das Doppelte der Rauheit (Ra) der keramischen Wärmesperrbeschichtung (1) beträgt,
- Anwenden der zirkonoxidbasierten Aufschlämmungsbeschichtung (2) mit der berechneten Anzahl von Spritzdurchgängen (N) auf die Oberfläche der keramischen Wärmesperrbeschichtung (1);
- vollständiges Härten, aber lediglich teilweises Sintern der zirkonoxidbasierten Aufschlämmungsbeschichtung (2) bei einer Temperatur im Bereich von 300 bis 800 °C;
- Polieren der zirkonoxidbasierten Aufschlämmungsbeschichtung (2); und
- vollständiges Sintern der zirkonoxidbasierten Beschichtung (2) erst nach der ersten Exposition zu einem wärmebelasteten Betrieb der Komponente (3); wobei der Polierschritt durchgeführt wird, bis die Spitzenwerte der Rauheit (Ra) erreicht werden, derart, dass die Dicke (T) der zirkonoxidbasierten Aufschlämmungsbeschichtung (2) eine verringerte Dicke (T') wird, die im Wesentlichen gleich der Rauheit (Ra) der keramischen Wärmesperrbeschichtung (1) ist, derart, dass schließlich die zirkonoxidbasierte Aufschlämmungsbeschichtung (2) die keramische Wärmesperrbeschichtung (1) lediglich lokal bei den Tälern der Rauheit (Ra) abdeckt.

2. Verfahren nach Anspruch 1, **gekennzeichnet durch** ein Härten bzw. teilweises Sintern der Aufschlämmungsbeschichtung (2) bei einer Temperatur im Bereich von 500 bis 800 °C.

3. Verfahren nach Anspruch 1, **dadurch gekennzeichnet, dass** das Zirkonoxid mit Y₂O₃, CaO, MgO oder einer beliebigen Kombination davon stabilisiert wird.

4. Verfahren nach Anspruch 1, **dadurch gekennzeichnet, dass** die keramische Wärmesperrbeschichtung (1) aus chemisch stabilisiertem Zirkonoxid hergestellt ist.

## Revendications

1. Procédé de réduction de la rugosité (Ra) d'un revêtement de type barrière thermique en céramique (1) ayant une composition de revêtement définie et un coefficient d'expansion thermique, ledit revêtement de type barrière thermique en céramique (1) recouvrant la surface d'un composant (3) de type superalliage à base de Ni, Co, Fe d'une turbine à gaz à forte sollicitation thermique, dans lequel :
- dans une première étape, le revêtement de type barrière thermique en céramique (1) est appliqué sur la surface d'un composant (3) par pulvérisation de plasma atmosphérique et la rugosité (Ra) dudit revêtement de type barrière thermique en céramique (1) est mesurée et
- dans une étape suivante, un revêtement liquide à base de zircone (2) avec des additifs de silicate d'alumine ou de silicate de zirconium et un liant de revêtement liquide qui est une solution de silicate, une solution de phosphate ou une émulsion de silicium est préparé pour une application sur la surface du revêtement de type barrière thermique en céramique (1), la composition de revêtement du revêtement liquide à base de zircone (2) étant adaptée pour avoir un coefficient d'expansion thermique similaire à celui du revêtement de type barrière thermique en céramique (1) ;
- calculer un nombre minimum de passages de pulvérisation de revêtement (N) nécessaires pour fournir le revêtement liquide à base de zircone (2) avec une épaisseur (T) qui est au moins deux fois la rugosité (Ra) du revêtement de type barrière thermique en céramique (1),
- appliquer le revêtement liquide à base de zircone (2) avec ledit nombre calculé de passages de pulvérisation (N) sur la surface du revêtement de type barrière thermique en céramique (1) ;
- durcir complètement, mais fritter uniquement partiellement le revêtement liquide à base de zircone (2) à une température comprise dans la plage allant de 300 à 800 °C ;
- polir le revêtement liquide à base de zircone (2) ;
- fritter totalement le revêtement liquide à base de zircone (2) uniquement après la première exposition à une opération de sollicitation thermique du composant (3) ;
l'étape de polissage est réalisée jusqu'à ce que les pics de rugosité (Ra) soient atteints de sorte que l'épaisseur (T) du revêtement liquide à base de zircone (2) devienne une épaisseur réduite (T') sensiblement égale à la rugosité (Ra) du revêtement de type barrière thermique en céramique (1) de sorte qu'en fin de compte le revêtement liquide à base de zircone (2) recouvre le revêtement de type barrière thermique en céramique (1) uniquement localement au niveau des vallons de rugosité (Ra).

2. Procédé selon la revendication 1, **caractérisé par** le durcissement puis le frittage partiel du revêtement liquide (2) à une température comprise dans la plage allant de 500 à 800 °C.

3. Procédé selon la revendication 1, caractérisé ce que la zircone est stabilisée avec de l'Y₂O₃, du CaO, du MgO ou n'importe quelle combinaison de ceux-ci.

4. Procédé selon la revendication 1, **caractérisé en ce que** le revêtement de type barrière thermique en céramique (1) se compose d'une zircone chimiquement stabilisée.
